

July 28, 1959

A. ZLETT ET AL

2,896,403

ROCKET PROPULSION METHOD

Filed Feb. 16, 1953



INVENTORS:  
Alex Zletz  
Don R. Carmody  
BY  
Michael Driscoll  
ATTORNEY

1

2,896,403

## ROCKET PROPULSION METHOD

Alex Zletz, Park Forest, and Don R. Carmody, Crete, Ill., assignors to Standard Oil Company, Chicago, Ill., a corporation of Indiana

Application February 16, 1953, Serial No. 336,906

16 Claims. (Cl. 60—35.4)

This invention relates to the generation of gas. More particularly, it relates to reaction propulsion by the hypergolic reaction of a liquid fuel and a liquid oxidizer. Still more particularly, the invention relates to a method of rocket propulsion by the hypergolic reaction of a fuel and a hydrogen peroxide oxidizer, which materials spontaneously react to generate gas at high pressure and high temperature.

Reaction propulsion is now being used for many aerial purposes. For many uses it is necessary to operate with a fuel system which is not dependent on atmospheric oxygen. This fuel system may consist of a single self-contained propellant or it may consist of a separate fuel and a separate oxidizer, i.e., a bipropellant system.

In the bipropellant system the fuel and the oxidizer are introduced separately and essentially simultaneously into the combustion chamber of the reaction motor. The products of oxidation from the reaction of the fuel and the oxidizer are discharged through an orifice at the exit end of the combustion chamber and thereby produce the driving force. Because of the possibilities of electrical and/or mechanical failure of the auxiliary methods of ignition such as a spark or a hot surface, it is preferred to use a self-igniting fuel system. A fuel which is self-igniting, i.e., spontaneously combustible when contacted with an oxidizer, is known as a hypergolic fuel.

Temperature has an important effect on the hypergolic activity of fuels. The temperature at the earth's surface may vary from a high of about +125° F. to a low of as much as —65° F.; in general temperatures below about —20° or —30° F. are exceptional. Thus surface-to-air missiles or rocket-driven aircraft should be capable of operation when the temperature of the fuel and the oxidizer at the moment of initial contact in the combustion chamber of the rocket motor is on the order of —20° F. Temperatures at high altitudes are frequently on the order of —65° F. and are known to approach —100° F. Thus an air-to-air missile should be able to operate satisfactorily when the temperature of the fuel and the oxidizer at the moment of initial contacting in the combustion chamber is on the order of —65° F.

The more common oxidizers are white fuming nitric acid, red fuming nitric acid and nitric acid-sulfuric acid mixtures. While these nitric acid oxidizers operate satisfactorily over a wide range of atmospheric temperatures they have important drawbacks. The nitric acid oxidizers are extremely corrosive; they have poor storage stability; they give off toxic gases; and special precautions must be taken by personnel who handle these oxidizers.

Concentrated aqueous hydrogen peroxide solutions have excellent storage stability and do not give off harmful gas. However, these aqueous hydrogen peroxide solutions such as 90% hydrogen peroxide have the disadvantage of freezing at +12° F. The freezing point of 80% hydrogen peroxide is —9° F., but the activity of this solution toward the prior art fuels is markedly lower than the 90% H<sub>2</sub>O<sub>2</sub> solution. The freezing point of aqueous hydrogen peroxide solu-

tions can be depressed by dissolving therein inorganic salts, preferably ammonium nitrate. Thus a solution containing 40 weight percent of ammonium nitrate and in which the hydrogen peroxide-water portion contains 5 90 weight percent of H<sub>2</sub>O<sub>2</sub> has a freezing point of about —30° F. A so-called 80% H<sub>2</sub>O<sub>2</sub>—30% NH<sub>4</sub>NO<sub>3</sub> solution has a freezing point of below —70° F.

Concentrated aqueous hydrogen peroxide solutions have been used as monopropellants by catalytically decomposing the hydrogen peroxide, using such catalysts as potassium permanganate or copper oxide. Since the decomposition products contain free-oxygen the monopropellant system is inefficient. However, fuels which are hypergolic with nitric acid oxidizers may be much less active or even inactive with concentrated H<sub>2</sub>O<sub>2</sub> solutions. Anhydrous hydrazine is usually considered to be the only fuel that is sufficiently hypergolic with concentrated H<sub>2</sub>O<sub>2</sub> solutions to be practical; however, hydrazine has the disability of a comparatively high freezing point. Some fuels are operative with H<sub>2</sub>O<sub>2</sub> solutions in the presence of a H<sub>2</sub>O<sub>2</sub> decomposition catalyst. Furthermore, the prior art fuels are less effective with ammonium nitrate containing H<sub>2</sub>O<sub>2</sub> than with H<sub>2</sub>O<sub>2</sub> alone.

An object of this invention is a method of generating gas by the hypergolic reaction of a fuel and a hydrogen peroxide oxidizer. Another object is a method of reaction propulsion by the hypergolic interaction of a fuel and a hydrogen peroxide oxidizer. Still another object is a method of reaction propulsion by the hypergolic interaction of a hydrogen peroxide oxidizer and a fuel which contains appreciable amounts of miscible hydrocarbons, particularly non-hypergolic liquid hydrocarbons. A particular object is a method of generating gas by the hypergolic interaction of a defined fuel and an oxidizer consisting of an aqueous hydrogen peroxide solution containing dissolved ammonium nitrate. Another particular object is a method of rocket propulsion by the hypergolic interaction of a defined organic phosphine and a defined hydrogen peroxide oxidizer when the temperature of the fuel and the oxidizer is about —70° F. Other objects will become apparent in the course of the detailed description of the invention.

A method has been discovered for generating gas, which gas may be used as a substitute for compressed air for certain purposes or for driving the turbine of a jet engine or for rocket propulsion, which method comprises contacting

- (1) A fuel consisting essentially of at least one member selected from the class consisting of
  - (A) Monoaliphaticmonohalophosphines which contain not more than 16 carbon atoms,
  - (B) Monoaliphaticdihalophosphines which contain not more than 10 carbon atoms, and
  - (C) Dialiphaticmonohalophosphines which contain not more than 12 carbon atoms and wherein each aliphatic radical contains not more than 8 carbon atoms, wherein the halogen radical in said phosphine is selected from the class consisting of chlorine and bromine, and
- (2) An oxidizer selected from the class consisting of
  - (i) Aqueous hydrogen peroxide solutions which contain at least about 60 weight percent of H<sub>2</sub>O<sub>2</sub> and the remainder is essentially water, and
  - (ii) Aqueous hydrogen peroxide-inorganic salt solutions wherein the hydrogen peroxide-water portion contains at least about 60 weight percent of H<sub>2</sub>O<sub>2</sub>.

The above phosphines can be blended with miscible hydrocarbon to produce hypergolic mixed fuels with

aqueous hydrogen peroxide solutions and, particularly, ammonium nitrate containing solutions suitable for operation at temperatures as low as  $-60^{\circ}$  F. The lower the initial temperature the less hydrocarbon tolerable in the blend.

Certain organic halophosphines ignite spontaneously when contacted with "hydrogen peroxide oxidizers." The various halophosphines do not have equal hypergolic activity with the same oxidizer. However, by proper selection of the halophosphine, it is possible to obtain a hypergolic reaction with a tolerable ignition delay when the phosphine and the oxidizer are at a temperature of about  $-70^{\circ}$  F. at the moment of initial contact in the gas generating chamber.

Certain monoaliphaticmonohalophosphines, monoaliphaticdihalophosphines, dialiphaticmonohalophosphines and mixtures thereof are useful for the purposes of this invention. These aliphatichalophosphines have the generic empirical formula RR'XP where P represents the element phosphorus, R represents an aliphatic radical, R' represents a radical selected from the class consisting of aliphatic hydrogen, chlorine and bromine, and X represents a radical selected from the class consisting of chlorine and bromine. The term "aliphatic" as used herein is intended to include hydrocarbon radicals selected from the class consisting of paraffins and olefins. It has been found that the highly branched aliphatic substituents have desirably lower freezing points than the straight chain or slightly branched substituents. It is preferred to use branched aliphatic substituents. The presence of unsaturated linkages in the aliphatic substituent improves the hypergolic activity. A particularly useful phosphine contains not only a highly branched aliphatic radical, but also contains one or more unsaturated linkages.

It has been found that the hypergolic activity of the various aliphatichalophosphines is dependent upon the number of aliphatic radicals, upon the total number of carbon atoms contained in the phosphine, and upon the number of carbon atoms contained in each of the aliphatic radicals. In order to obtain a fuel which is usable at low temperatures, it is necessary that the monoaliphaticmonohalophosphines contain not more than 16 carbon atoms. The monoaliphaticdihalophosphines must contain not more than 10 carbon atoms in the molecule. The dialiphaticmonohalophosphines must not contain more than 12 carbon atoms in the molecule and furthermore, no aliphatic radical must contain more than 8 carbon atoms.

Each halophosphine of this invention must contain at least one, and preferably two, halogen radicals selected from the class consisting of chlorine and bromine.

When it is desired to initiate the combustion at very low atmospheric temperatures, i.e., about  $-60$  or  $-70$  F., it is preferred to use the following fuels: monoalkyl-dihalophosphines which contain not more than 4 carbon atoms and dialkylmonohalophosphines which contain not more than 6 carbon atoms and wherein each alkyl radical contains not more than 4 carbon atoms. The preferred species for operation at starting temperatures of about  $-70$  F. are the monoethylchlorophosphine, diethylmonochlorophosphine and dimethylmonobromophosphine.

A mixed fuel which is suitable for the generation of gas for reaction propulsion when the fuel and the oxidizer are at a temperature of about  $-60$  F. can be made by mixing an alkyl halophosphine with a miscible hydrocarbon. An effective amount of halophosphine must necessarily be present in the mixed fuel in order to obtain the hypergolic reaction. This amount will vary with both the type of hydrocarbon and the species of halophosphine. When using a monoethylchlorophosphine and aromatic hydrocarbon mixture, as much as 60 volume percent of the mixed fuel may be aromatic hydrocarbons, for operations at temperatures of above

about  $+60$  F. For operation at temperatures of about  $-60$  F., only about 25 volume percent of hydrocarbon is tolerable in the blend. In general, the higher the initial temperature of the fuel and the oxidizer, the more hydrocarbon tolerable in the mixed fuel. In general petroleum hydrocarbon fractions are suitable materials, for example, those fractions boiling between about  $300^{\circ}$  and  $600^{\circ}$  F. which correspond to the fuel requirement of military jet engines. Aromatic hydrocarbons which boil below about  $600^{\circ}$  F. are suitable hydrocarbons for this purpose. The low temperature hypergolic activity of the mixed fuel can be improved by using as the hydrocarbon component olefinic hydrocarbons such as thermal-cracked naphthas and gas oils or turpentine.

The oxidizers of this invention may be either concentrated aqueous hydrogen peroxide solutions or aqueous hydrogen peroxide solutions containing dissolved inorganic salts, for example, ammonium halides, sodium sulfate, sodium nitrate, etc.; for low temperature operation which requires a short ignition delay, ammonium nitrate must be used as the inorganic salt. The concentrated aqueous hydrogen peroxide solutions should contain at least about 60 weight percent of  $H_2O_2$ ; the remainder of the solution is essentially water.

The hypergolic activity of the aqueous hydrogen peroxide solution is improved by increasing the concentration of the peroxide. Commercially available 90%  $H_2O_2$  solution is an excellent oxidizer for operation at temperatures above about  $0^{\circ}$  F. For operation at temperatures below about  $0^{\circ}$  F., it is preferred to use aqueous  $H_2O_2$ -ammonium nitrate solutions, such as, "90%-40%" or "80%-30%" solutions.

Concentrated aqueous hydrogen peroxide solution as made commercially is virtually only  $H_2O_2$  and water. In order to improve storage stability small amounts of stabilizers may be added to the solution, e.g., sodium stannate, tetrasodium pyrophosphate, adipic acid, tartaric acid; in general only trace amounts of stabilizers are added so that the solution consists essentially of hydrogen peroxide and water.

In order to depress the freezing point of aqueous hydrogen peroxide solutions soluble inorganic salts are dissolved therein, e.g., sodium nitrate, ammonium chloride and ammonium nitrate have been used. These salt-containing solutions are commonly designated in terms of the weight percent of salt in the total solution and the weight percent of hydrogen peroxide present in the aqueous portion of the solution, e.g., 90%  $H_2O_2$ -40%  $NH_4NO_3$  indicates that the total aqueous hydrogen peroxide-nitrate solution consists of 40 weight percent of ammonium nitrate and 60 weight percent of aqueous hydrogen peroxide composed of 90 weight percent of  $H_2O_2$  and the remainder essentially water. This particular solution has a freezing point of about  $-30^{\circ}$  F. A temperature of  $-70^{\circ}$  F. is attainable with an 80%  $H_2O_2$ -30%  $NH_4NO_3$  solution. It is preferred to operate in the presence of ammonium nitrate because of the pronounced favorable effect on the hypergolic activity of the fuels of this invention.

It has previously been found that monoaliphaticphosphines which contain between 1 and 16 carbon atoms, dialiphaticphosphines which contain between 2 and 20 carbon atoms and wherein each aliphatic radical contains between 1 and 12 carbon atoms, and trialiphaticphosphines which contain between 3 and 24 carbon atoms and wherein each aliphatic radical contains between 1 and 12 carbon atoms are hypergolic with aqueous hydrogen peroxide oxidizers containing about 90%  $H_2O_2$  at temperatures above about  $-20^{\circ}$  F. Examples of these fuels are: tributylphosphine, dodecylphosphine and dioctylphosphine. The hypergolic activity of these fuels at lower temperatures can be greatly improved by adding thereto small amounts of the above defined halophosphines, i.e., the halophosphines have a synergistic catalytic effect on the activity of aliphatic phosphines. For low temperatures the halophosphine-phosphine fuel should contain between about 1 and 15

volume percent of halophosphine, preferably the dihalophosphine.

Monoethyldichlorophosphine ( $C_2H_5PCl_2$ ) was prepared by the method of Karasch, Jensen and Weinhaus, J. Org. Chem., 14, 429 (1949) using 137 g. of  $PCl_3$  and 100 g. of lead tetraethyl. The two reagents were heated for 11 hours in a nitrogen atmosphere under total reflux; the reflux temperature rose from 85° C. to 118° C. A 35% yield was obtained of a fraction boiling between 112-122° C. at 750 mm. pressure. The literature boiling point of monoethyldichlorophosphine is 114-117° C.

The ignition characteristics of various fuels were studied using a "drop" test. This method utilizes a test tube, 1 in. x 4 in., containing about 0.5 ml. of oxidizer. The fuel to be tested was drawn into a hypodermic syringe. It was then ejected forcefully against the oxidizer surface by depressing the syringe plunger. By this method amounts of fuel of as little as 0.01 ml. can be added. Low temperature tests were carried out by cooling the test tube and the oxidizer contained therein by means of a bath; a drying tube inserted into the top of the test tube excluded moisture. The fuel was cooled separately to the desired test temperature. By supercooling it was possible to carry out tests at temperatures below the freezing point of the fuel and/or the oxidizer.

The "ignition delay," which is the time elapsing between the addition of fuel to the oxidizer and visual ignition thereof, was determined visually as either (a) very short which corresponds to substantially instantaneous ignition, (b) short, which corresponds to substantially less than 1 second, and (c) more than 1 second, which time was determined by a stop watch.

The following tests illustrate the activity of some of the alkyl halophosphines of this invention and hydrazine with hydrogen peroxide oxidizers.

#### Test 1

In this test several runs were made with monoethyldichlorophosphine at different temperatures using 0.5 ml. of various  $H_2O_2$  solutions as the oxidizer. A run was made with mono(n-octyl)phosphine for comparison purposes.

| Run No. | Fuel | Fuel added, ml. | $H_2O_2$ Oxidizer, percent | Temp., °F. | Ignition delay |
|---------|------|-----------------|----------------------------|------------|----------------|
| 1.      | (a)  | 0.01            | 90                         | +70        | Very short.    |
| 2.      | (a)  | 0.02            | 90                         | -6         | Short.         |
| 3.      | (a)  | 0.03            | 90                         | -24        | Do.            |
| 4.      | (a)  | 0.02            | 80                         | -6         | Do.            |
| 5.      | (a)  | 0.04            | 80                         | -24        | Do.            |
| 6.      | (a)  | 0.10            | 60                         | -20        | 2 sec.         |
| 7.      | (b)  | 0.08            | 80                         | -20        | 2 sec.         |

<sup>a</sup> Monoethyldichlorophosphine.

<sup>b</sup> Mono(n-octyl)phosphine.

These data show that the halophosphines are much more hypergolic than are the alkylphosphines.

#### Test 2

In order to observe the effectiveness of halophosphine with oxidizers consisting of aqueous hydrogen peroxide-ammonium nitrate solutions, runs were made using 0.5 ml. of aqueous hydrogen peroxide-ammonium nitrate solutions as the oxidizer, and monoethyldichlorophosphine as the fuel.

| Run No. | Fuel | Fuel added, ml. | Oxidizer $H_2O_2$ - $NH_4NO_3$ , percent | Temp., °F. | Ignition delay               |
|---------|------|-----------------|------------------------------------------|------------|------------------------------|
| 8.      | (a)  | 0.03            | 90-40                                    | -40        | Very short.                  |
| 9.      | (a)  | 0.06            | 80-30                                    | -60        | Short.                       |
| 10.     | (a)  | 0.10            | 80-30                                    | -72        | Do.                          |
| 11.     | (a)  | 0.15            | 80-30                                    | -82        | No ignition (effervescence). |
| 12.     | (b)  | 0.02            | 90-40                                    | +70        | 2 sec.                       |

<sup>a</sup> Monoethyldichlorophosphine.

<sup>b</sup> Mono(n-octyl)phosphine.

These data show how enormously more effective the halophosphines are with nitrate containing  $H_2O_2$  oxidizers, than are the alkylphosphines.

#### Test 3

For comparative purposes hydrazine was contacted at various temperatures with either 90%  $H_2O_2$  or 80%  $H_2O_2$  solutions as the oxidizer.

| Run No.         | $H_2O_2$ oxidizer, percent | Fuel added, ml. | Temp., °F. | Ignition delay               |
|-----------------|----------------------------|-----------------|------------|------------------------------|
| 13.             | 90                         | 0.05            | +70        | Very short.                  |
| 14.             | 80                         | 0.03            | +70        | Short.                       |
| 15.             | 80                         | 0.10            | +14        | No ignition (effervescence). |
| 16 <sup>a</sup> | 90                         | 0.03            | +14        | Very short.                  |
| 16.             | 90-40                      | 0.03            | +14        | No ignition.                 |

#### Test 4

The hypergolic activity of mixtures of toluene and monoethyldichlorophosphine was tested at various blends and various temperatures using 0.5 ml. of various oxidizers.

| Run No. | Toluene content, vol. percent | Fuel added, ml. | Oxidizer $H_2O_2$ - $NH_4NO_3$ , percent | Temp., °F. | Ignition delay                                                   |
|---------|-------------------------------|-----------------|------------------------------------------|------------|------------------------------------------------------------------|
| 17.     | 22                            | 0.02            | 90                                       | +70        | Very short.                                                      |
| 18.     | 30                            | 0.06            | 90                                       | +70        | Do.                                                              |
| 19.     | 40                            | 0.06            | 90                                       | +70        | Do.                                                              |
| 20.     | 40                            | 0.12            | 90                                       | +70        | Do.                                                              |
| 21.     | 50                            | 0.20            | 90                                       | +70        | Do.                                                              |
| 22.     | 22                            | 0.02            | 90-40                                    | +70        | Do.                                                              |
| 23.     | 22                            | 0.04            | 90                                       | 0          | 2 sec.                                                           |
| 24.     | 22                            | 0.07            | 90                                       | 0          | Do.                                                              |
| 25.     | 22                            | 0.06            | 90-40                                    | -42        | Very short.                                                      |
| 26.     | 22                            | 0.03            | 80                                       | +70        | Do.                                                              |
| 27.     | 22                            | 0.07            | 80                                       | -2         | 4 sec.                                                           |
| 28.     | 50                            | 0.10            | 90                                       | +70        | Mono (n-octyl) phosphine and benzene were tested for comparison. |
| 29.     | 50                            | 0.15            | 90                                       | +70        | No ignition.                                                     |
|         |                               |                 |                                          |            | Short.                                                           |

These runs show the greater hypergolic activity of the halophosphine-aromatic hydrocarbon mixed fuels over the alkylphosphine mixed fuels.

#### Test 5

The effect on activity of the presence of various salts in the hydrogen peroxide oxidizer was studied using as the fuel a blend of toluene, 25 vol. percent, and ethyl-dichlorophosphine, 75 vol. percent, and 0.5 ml. of oxidizer.

| Run No. | Mixed fuel added, ml. | Oxidizer | Temp., °F. | Ignition delay           |
|---------|-----------------------|----------|------------|--------------------------|
| 30.     | 0.07                  | (1)      | -3         | Short.                   |
| 31.     | 0.07                  | (2)      | -3         | Very short.              |
| 32.     | 0.07                  | (2)      | -5         | Do.                      |
| 33.     | 0.07                  | (3)      | -5         | No ignition.             |
| 34.     | 0.07                  | (4)      | -5         | No ignition (vig. eff.). |

<sup>1</sup> 80%  $H_2O_2$ .

<sup>2</sup> 80%  $H_2O_2$ -20%  $NH_4NO_3$ .

<sup>3</sup> 80%  $H_2O_2$ -20%  $NH_4Cl$ .

<sup>4</sup> 80%  $H_2O_2$ -sat'd.  $NaNO_3$  (would not dissolve 20% of salt).

These runs show the extremely favorable effect on activity of ammonium nitrate in the hydrogen peroxide oxidizer.

It is obvious from the data presented above that this invention can be used to generate gas at high pressure. This gas can be used for operating machinery such as "compressed air hammers" or for aircraft catapults; another important use for this high pressure gas is in the starting of the turbines of jet-type engines. The invention is particularly useful for operations which require a compact power plant that is able to produce a large amount of energy over a very short period of time, when the fuel and oxidizer are at low atmospheric tempera-

tures. Other examples of uses of this invention are: the rocket-assisted takeoff or flight of aircraft; aerial missiles; boosters for surface vehicles.

The relative proportion of oxidizer-to-fuel used will depend upon the type of operation, the temperature of operation and the type of fuel and oxidizer being used. When using a "80%  $H_2O_2$ -30%  $NH_4NO_3$ " solution as the oxidizer and dibutylmonochlorophosphine as the fuel, between about 4 and 5 volumes of oxidizer are needed per volume of fuel.

By way of example this invention is applied to the propulsion of a surface-to-air missile. The annexed figure which forms a part of this specification shows schematically the bipropellant feed system and the motor of this missile. This same type of missile could be used as an air-to-air missile. This missile is suitable for operations wherein the fuel and the oxidizer can be maintained at a temperature high enough to insure at least a short ignition delay, e.g., when using the above oxidizer and fuel combination, a temperature of about  $-70^\circ F$ .

In the drawing vessel 11 contains a quantity of gas at high pressure; this gas must be inert with respect to the oxidizer and the fuel; suitable gases are nitrogen and helium. Herein helium is used as the inert gas. Helium from vessel 11 is passed through line 12 and through valve 13 which regulates the flow of gas to maintain a constant pressure beyond valve 13. From valve 13 helium is passed through lines 14 and 16 into vessel 17 and simultaneously through line 18 into vessel 19.

Vessel 17 contains the oxidizer. Helium pressure forces the oxidizer out of vessel 17 through line 21 to valve 22. Valve 22 is a solenoid actuated throttling valve. Suitable electrical lines connect valve 22 to an electrical source and operating switch (not shown) at the control chamber at the launching site. The oxidizer is passed through line 23 and injector 24 into combustion chamber 26. Combustion chamber 26 is provided with an outlet nozzle 27.

Vessel 19 contains the fuel. Vessels 17 and 19 are constructed to withstand the high pressure imposed by the helium gas. The gas pressure forces fuel from vessel 19 through line 28 to solenoid actuated throttling valve 29. Valve 29 is similar in construction and in actuation to valve 22. The fuel is passed through line 31 and injector 32 into combustion chamber 26.

Valves 22 and 29 are of such a size and setting that a predetermined ratio of oxidizer-to-fuel is passed into combustion chamber 26. Injectors 24 and 32 are so arranged that the streams of oxidizer and fuel converge and contact each other forcibly, resulting in a very thorough intermingling of the fuel and the oxidizer.

The missile is launched by activating the solenoids on valves 22 and 29. In this example 4.2 volumes of 80%-30% solution per volume of halophosphine is introduced into the combustion chamber. The oxidizer and the fuel react almost instantaneously upon contact in the combustion chamber; a large volume of very hot gas is produced in the combustion chamber, which gas escapes through orifice 27. The reaction from this expulsion of gas drives the missile toward its target.

Thus having described the invention, what is claimed is:

1. A method of generating gas, which method comprises injecting separately and essentially simultaneously into the combustion chamber of a gas generator (1) a hypergolic fuel consisting essentially of a member selected from the class consisting of (i) monoorganicmono-halophosphines containing not more than 16 carbon atoms, (ii) monoorganicdihalophosphines containing not more than 10 carbon atoms and (iii) diorganicmono-halophosphines containing not more than 12 carbon atoms and not more than 8 carbon atoms in an organic group, wherein the organic groups in (i), (ii) and (iii) above are alkyl and the halogen radicals are selected from the class consisting of chlorine and bromine and

(2) an oxidizer selected from the class consisting of (a) aqueous hydrogen peroxide solutions consisting of at least about 80 weight percent of  $H_2O_2$  and the remainder essentially water and (b) aqueous hydrogen peroxide-ammonium nitrate solutions wherein the hydrogen peroxide-water portion is the predominant component and consists of at least about 80 weight percent of  $H_2O_2$  and the remainder essentially water, in an amount and at a rate sufficient to initiate a hypergolic reaction with and to support combustion of the fuel.

2. The method of claim 1 wherein said fuel is monoethyl dichlorophosphine.

3. The method of claim 1 wherein said fuel is dibutyl monochlorophosphine.

4. The method of claim 1 wherein said fuel is diethyl monochlorophosphine.

5. The method of claim 1 wherein said oxidizer consists of about 80 weight percent of  $H_2O_2$  and the remainder essentially water.

6. The method of claim 1 wherein said oxidizer consists of about 90 weight percent of  $H_2O_2$  and the remainder essentially water.

7. The method of claim 1 wherein said oxidizer consists of a solution of hydrogen peroxide, water and ammonium nitrate, wherein the nitrate content is about 30 weight percent and the hydrogen peroxide-water portion consists of about 80 weight percent of  $H_2O_2$  and the remainder essentially water.

8. The method of claim 1 wherein said oxidizer consists of a solution of hydrogen peroxide, water and ammonium nitrate, wherein the nitrate content is about 40 weight percent and the hydrogen peroxide-water portion consists of about 90 weight percent of  $H_2O_2$  and the remainder essentially water.

9. A method of generating gas, which method comprises injecting separately and essentially simultaneously into the combustion chamber of a gas generator (1) a hypergolic mixed fuel consisting essentially of (I) a liquid miscible hydrocarbon and (II) monoethyl dichlorophosphine and (2) an oxidizer selected from the class consisting of (a) aqueous hydrogen peroxide solutions consisting of at least about 80 weight percent of  $H_2O_2$  and the remainder essentially water, and (b) aqueous hydrogen peroxide-ammonium nitrate solutions wherein the hydrogen peroxide-water portion is the predominant component and consists of at least about 80 weight percent of  $H_2O_2$  and the remainder essentially water, in an amount and at a rate sufficient to initiate a hypergolic reaction with and to support combustion of the mixed fuel.

10. The method of claim 9 wherein said hydrocarbon is a liquid petroleum fraction boiling between about 300° and about 600° F.

11. The method of claim 9 wherein said hydrocarbon is a liquid aromatic hydrocarbon boiling below about 600° F.

12. The method of claim 9 wherein said hydrocarbon is a liquid olefin boiling below about 600° F.

13. A method of generating gas, which method comprises injecting separately and essentially simultaneously into the combustion chamber of a gas generator (1) a hypergolic mixed fuel consisting essentially of (I) a liquid miscible hydrocarbon and (II) diethyl monochlorophosphine and (2) an oxidizer selected from the class consisting of (a) aqueous hydrogen peroxide solutions consisting of at least about 80 weight percent of  $H_2O_2$  and the remainder essentially water, and (b) aqueous hydrogen peroxide-ammonium nitrate solutions wherein the hydrogen peroxide-water portion is the predominant component and consists of at least about 80 weight percent of  $H_2O_2$  and the remainder essentially water, in an amount and at a rate sufficient to initiate a hypergolic reaction with and to support combustion of the mixed fuel.

14. A method of gas generation, which method comprises injecting separately and essentially simultaneously

into the combustion chamber of a gas generator (1) a hypergolic fuel consisting essentially of (A) alkyl phosphines selected from the class consisting of (i) mono-alkylphosphines containing not more than 16 carbon atoms, (ii) dialkylphosphines containing not more than 20 carbon atoms and not more than 12 carbon atoms in an alkyl radical, and (iii) trialkylphosphines containing not more than 24 carbon atoms and not more than 12 carbon atoms in an alkyl radical, and (B) between about 1 and 15 volume percent based on fuel of a halophosphine selected from the class consisting of (i) mono-organicmonohalophosphines containing not more than 16 carbon atoms (ii) monoorganicdihalophosphines containing not more than 10 carbon atoms and (iii) diorganic-monohalophosphines containing not more than 12 carbon atoms and not more than 8 carbon atoms in an organic group, wherein the organic groups in (i), (ii) and (iii) above are alkyl and the halogen radicals are selected from the class consisting of chlorine and bromine and (2) an oxidizer selected from the class consisting of (a) aqueous hydrogen peroxide solutions consisting of at least about 80 weight percent of  $H_2O_2$  and the re-

mainder essentially water and (b) aqueous hydrogen peroxide-ammonium nitrate solutions, wherein the hydrogen peroxide-water portion is the predominant component and consists of at least about 80 weight percent of  $H_2O_2$  and the remainder essentially water, in an amount and at a rate sufficient to initiate a hypergolic reaction with and to support combustion of the fuel.

15. The method of claim 14 wherein said halophosphine is monoethylchlorophosphine.

16. The method of claim 14 wherein said aliphatic phosphine is tributylphosphine.

References Cited in the file of this patent

FOREIGN PATENTS

15 673,451 Great Britain ----- June 4, 1952

OTHER REFERENCES

Hackh's Chemical Dictionary, 3rd Edition (1944).  
The Blakiston Co., Philadelphia, Pa., page 559.

20 Kavash et al.: "Journal Org. Chem.", vol. 14 (1949),  
p. 429.